# EUROPEAN PATENT SPECIFICATION

(11) **EP 1 595 969 B1**
(45) Date of publication and mention of the grant of the patent: **28.06.2017**
(21) Application number: 04708495.9
(22) Date of filing: 05.02.2004
(51) Int. Cl.: C23C 2/06, C23C 2/28

(54) **GALVANNEALED STEEL SHEET EXCELLENT IN COATING ADHESION AND MANUFACTURING METHOD THEREOF**
NACH DEM HEISSTAUCHVERFAHREN MIT LEGIERTEM ZINK BESCHICHTETES STAHLBLECH MIT HERVORRAGENDER HAFTUNG UND HERSTELLUNGSVERFAHREN DAFÜR
TÔLE D'ACIER PLAQUÉE PAR IMMERSION À CHAUD DANS UN ALLIAGE DE ZINC PRÉSENTANT UNE EXCELLENTE ADHÉRENCE ET PROCÉDÉ DE PRODUCTION

(30) Priority: 10.02.2003 JP 2003032321; 10.02.2003 JP 2003032311; 10.02.2003 JP 2003032500; 21.01.2004 JP 2004013269
(43) Date of publication of application: 16.11.2005
(73) Proprietor: JFE Steel Corporation, Tokyo, 100-0011 (JP)
(72) Inventor: TADA, Masahiko c/o Int. P. Dept. JFE Steel Corp., Chiyoda-ku Tokyo 100-0011 (JP); TOBIYAMA, Yoichi Int. P. Dept. JFE Steel Corp., Chiyoda-ku Tokyo 100-0011 (JP); KYONO, Kazuaki Int. P. Dept. JFE Steel Corp., Chiyoda-ku Tokyo 100-0011 (JP); MAKIISHI, Noriko Int. P. Dept. JFE Steel Corp., Chiyoda-ku Tokyo 100-0011 (JP); NORO, Hisato Int. P. Dept. JFE Steel Corp., Chiyoda-ku Tokyo 100-0011 (JP)
(74) Representative: Henkel, Breuer & Partner
(86) International application number: PCT/JP2004/001209
(87) International publication number: WO 2004/070075

(56) References cited:
- JP-A- 5 263 207
- JP-A- 7 034 213
- JP-A- 10 096 064
- JP-A- 2000 290 730
- JP-A- 2001 303 226
- NAKAMORI T ET AL: "Coating adhesion and interface structure of galvannealed steel" ISIJ INTERNATIONAL, vol. 35, no. 12, 1995, pages 1494-1501, XP002560972 IRON AND STEEL INSTITUTE OF JAPAN, TOKYO [JP]
- TOKI T ET AL: "The effect of Si in steel on adhesion strength of galvannealed steel" TETSU TO HAGANE: JOURNAL OF THE IRON AND STEEL INSTITUTE OFJAPAN, vol. 89, no. 1, 1 January 2003 (2003-01-01), pages 46-53, XP009127314 IRON AND STEEL INSTITUTE OF JAPAN, TOKYO [JP] ISSN: 0021-1575
- BORDIGNON L ET AL: "Enhanced hot dip galvanising by controlled oxidation in the annealing furnace" 44TH MWSP (MECHANICAL WORKING AND STEEL PROCESSING) CONFERENCE PROCEEDINGS, ORLANDO, FL [US] 8 - 11 SEPTEMBER 2002 vol. XL, September 2002 (2002-09), pages 833-844, XP002560973 Centre for Research in Metallurgy (CRM), Liège [BE] Retrieved from the Internet: URL:http://www.crm-eur.com/F-PUBLICATIONS/ media/2002/ENHANCED.PDF> [retrieved on 2009-12-15]

## Description

### Technical Field

The present invention relates to a galvannealed steel sheet excellent in the coating adhesion to a base steel sheet (mother material) and a method or manufacturing the same.

### Background Art

In recent years, in the fields of automobiles, home electric appliances and construction materials, steel sheets that are surface treated to impart the rust resistance to base steel sheets are used. Among these, galvannealed steel sheets that can be cheaply manufactured and are excellent in the rust resistance after coating are in use. In the field of automobiles in particular, higher mechanical strength and lighter weight of the base steel sheets are in progress. There is an increasing tendency in the use of more galvannealed steel sheets that are rust resistant and high in the mechanical strength.

However, since an interface between a coating layer and a base steel sheet of a galvannealed steel sheet is brittle, for instance, when it is press-molded with a die, the coating layer peels, and the peeled coating layer sticks to the die to deteriorate product quality; accordingly, frequent cleaning of the die is necessary. In some cases, at a portion adhered with a secondary material, the coating layer peels and desired adhesive strength cannot be obtained. Alternatively, there is a problem in that when an automobile is running in winter, a coating layer comes to peel owing to chipping due to splattered stones or the like, and thereby desired rust resistance cannot be maintained.

In general, a galvannealed steel sheet, after a surface of a base steel sheet is degreased and/or acid washed to cleanse in a pretreatment process or, without applying the pre treatment, an oil content on a surface of the base steel sheet is burned and removed in a pre-heating furnace, is preheated in a weak acidic or reducing atmosphere, and undergoes a recrystallization annealing process in a reducing atmosphere . Thereafter, the base steel sheet is cooled in a reducing atmosphere to a temperature suitable for the coating, without exposing to air, dipped in a molten zinc coating bath in which a slight amount of Al (substantially 0.1 to 0.2 mass percent) is added, followed by controlling a coating thickness, and thereby a galvannealed steel sheet is manufactured.

A coating layer of the galvannealed steel sheet is made of an Fe-Zn alloy phase that is formed through mutual diffusion of Fe and Zn. In the neighborhood of an interface between the coating layer and the base steel sheet, an Fe-Zn alloy phase rich in a content of Fe is formed, and, as coming closer toward a surface of the coating layer, an Fe-Zn alloy phase poor in the content of Fe is formed. Since the Fe-Zn alloy phase that is formed in the neighborhood of an interface between the coating layer and the base steel sheet and rich in the content of Fe (for instance, Γ phase and Γ1 phase) is hard and brittle, when it is formed excessively thicker, the brittleness at the interface between the coating layer and the base steel sheet is enhanced. Furthermore, because the coating layer of the galvannealed steel sheet is made of an Fe-Zn alloy phase, there is a disadvantage in that since the adhesion of the coating layer at the interface between the coating layer and the base steel sheet is poor, peeling at the interface between the coating layer and the base steel sheet is likely to occur.

So far, in the galvannealed steel sheets, a method of improving the coating adhesion with the base steel sheet has been variously studied. For instance, in Patent Document 1, a technique in which in the case of ultra low carbon IF steel (Interstitial Free Steel) that contains 0.006 mass percent or less of carbon being used as a mother material, when Si, P and so on are properly added to steel, Zn in the coating layer is promoted to diffuse into a grain boundary of the mother material, and thereby the coating adhesion is improved is disclosed. However, in recent demands for higher mechanical strength, the ultra low carbon IF steel, being low in the mechanical strength, cannot attain satisfying performance. Furthermore, there is a problem in that in the case of a high strength steel sheet (for instance, a steel sheet in which carbon and other alloying elements are contained much in a mother material, thereby the tensile strength is made 440 MPa or more) being used, the technique according to the Patent Document 1 cannot necessarily obtain satisfying adhesiveness of the coating layer.

In Patent Document 2, it is disclosed that in the case of P-added steel in which 0.010 to 0.10 mass percent of P and 0.05 to 0.20 mass percent of Si are added to a mother material and Si ≥ P is satisfied being used, the adhesion of the coating can be improved. However, in the case of the technique being applied to steel sheets other than the P-added steel sheet, there is a problem in that satisfying adhesion of the coating layer cannot be necessarily obtained.

Furthermore, in Patent Document 3, a technique in which in the case of high strength retained austenite steel in which low carbon steel containing 0.05 to 0.25 mass percent of carbon is used as a mother material and proper amounts of Si and Al are added, when proper amounts of Ti, Nb and so on are added in the steel to fix interstitial C, the coating interface strength can be improved is disclosed. However, this is a technique of the retained austenite steel, and there is a problem in that according to the technique described in Patent Document 3, in other high strength steel sheets that do not have a retained austenite phase, sufficient performance cannot be necessarily obtained.

Still furthermore, so far, as to a technique of improving the adhesion of an interface between a coating layer and a steel sheet of a galvannealed steel sheet, various studies have been conducted while paying attention to a shape of an interface between the coating layer and the base steel sheet. For instance, in Patent Documents 4 and 5, a technique in which the surface roughness of a surface of a steel sheet after a coating layer is removed therefrom is made 6.5 µm or more in terms of ten point height of irregularities Rz is disclosed. Furthermore, in Patent Document 6, a technique in which of P-added steel, the surface roughness Rz of a surface of the steel after a coating layer is removed therefrom is made to satisfy 12 ≥ Rz ≥ 0.0075 - Sm + 6.7 (where, Rz (µm): ten point height of irregularities, and Sm (µm) : average distance between irregularities) is disclosed. However, the present inventors, after studying hard, found a new finding in that in a shape of an interface between the coating layer and the base steel sheet that contributes to the coating adhesion, fine irregularities that cannot be defined with the ten point height of irregularities Rz that is used in the existing finding are important, and thereby a galvannealed steel sheet very excellent in the coating adhesion to an extent that has not been so far found can be obtained.

Non-Patent Document 1 relates to enhanced hot dip galvanising by controlled oxidation in the annealing furnace. In this context, a number of galvannealed steel sheets comprising a galvannealed layer formed on a base steel sheet are disclosed, wherein the base steel sheet may be derived from a steel containing, in % by mass, 0.0035% of C, 0.154% of Si, 0.072% of P, 0.043% of Ti, 0.019% of Nb, 0.589% of Mn, 0.029% of Al, and 0.022% of Cr.
Patent Document 1: Japanese Patent No. 3163986
Patent Document 2: Japanese Patent No. 2993404
Patent Document 3: JP-A-2001-335908
Patent Document 4: Japanese Patent No. 2638400
Patent Document 5: Japanese Patent No. 2932850
Patent Document 6: Japanese Patent No. 2976845

Non-Patent Document 1: Bordignon et al., 44th MWSP Conference Proceedings, Orlando, September 2002, Vol. XL, 2002, 833-844

### Disclosure of Invention

The present invention intends to provide a galvannealed steel sheet that is remarkably excellent in the coating adhesion in comparison with an existing product, and a manufacturing method thereof. The invention is defined by the claims.

In a first aspect, the present invention thus relates to a galvannealed steel sheet excellent in the coating adhesion, the galvannealed steel sheet comprising a galvannealed layer which is formed on a base steel sheet that
(i) contains, in % by mass, 0.25% or less of C, 0.03 to 2.0% of Si, 0.005 to 0.07% of P, and at least one kind selected from 0.2% or less of Ti, 0.2% or less of Nb and 0.2% or less of V, and
(ii) has a composition satisfying both the equation [C] + [P] ≤ [Si] and the equation [Ti] + [Nb] + [V] ≥ [P], with [C], [Si], [P], [Ti], [Nb] and [V], respectively, meaning the contents (% by mass) of C, Si, P, Ti, Nb and V in the base steel sheet,
wherein, in an interface between the galvannealed layer and the base steel sheet, an irregular portion that has a depth of 10 nm or more at a pitch of 0.5 µm or less is present at least one per 5 µm of a length of the interface, as determined by scanning electron microscopy together with transmission electron microscopy, the depth being defined as the distance in a straight line measured in a height direction between a base that is at a position lowest in height within a reference length and the lower one of a first top and a second top that are at positions highest in height on each of both sides of the base within the reference length, and the pitch being defined as the distance in a straight line measured in a length direction between the first top and the second top within the reference length,
and wherein the base steel sheet contains an oxide of silicon immediate below the interface.

In a second aspect, the present invention relates to a method of manufacturing a galvannealed steel sheet as defined in the first aspect, the method comprising the steps of:
(a) heat-treating a base steel sheet that
   (i) contains, in % by mass, 0.25% or less of C, 0.03 to 2.0% of Si, 0.005 to 0.07% of P, and at least one kind selected from 0.2% or less of Ti, 0.2% or less of Nb and 0.2% or less of V, and
   (ii) has a composition satisfying both the equation [C] + [P] ≤ [Si] and the equation [Ti] + [Nb] + [V] ≥ [P], with [C], [Si], [P], [Ti], [Nb] and [V], respectively, meaning the contents (% by mass) of C, Si, P, Ti, Nb and V in the base steel sheet,
   in an atmosphere containing 0.01 to 0.5% by volume of oxygen, having a dew point in the range of -20 to +20°C, the balance being made of nitrogen, and having a temperature in the range of 300 to 500°C so that Si in the steel is not selectively surface oxidized,
(b) heat-treating the base steel sheet obtained from step (a) in a reducing atmosphere containing 3 to 20% by volume of hydrogen, the balance being made of nitrogen, at a temperature in the range of from 750 to 900°C,
(c) cooling the base steel sheet obtained from step (b) to a coating temperature in an atmosphere having an oxygen concentration of 0.005% by volume or less,
(d) dipping the base steel sheet obtained from step (c) in a molten zinc coating bath to form a coating layer, and
(e) heating the base steel sheet obtained from step (d) at a temperature rise speed of 20°C/s or more to a temperature range of 460 to 600°C and holding in the heating temperature range to apply a galvannealing process of the coating layer, wherein the temperature rise speed and the content of Si in the base steel sheet satisfy the equation ST ≥ 3.25/[Si], with ST designating the temperature rise speed (°C/s) and [Si] designating the content (% by mass) of Si in the base steel sheet.

### Brief Description of the Drawings

Fig. 1 is a SEM photograph, in a galvannealed steel sheet according to the present invention, of a surface of a steel sheet after a coating layer is dissolved and removed.
Fig. 2 is a cross sectional SEM photograph of the galvannealed steel sheet according to the invention.
Fig. 3 is a diagram for explaining fine irregularities formed at an interface between a coating layer and a steel sheet in a galvannealed steel sheet according to the present invention.
Fig. 4 is a graph showing relationship between a ratio with which fine irregularities formed at an interface between the coating layer and the steel sheet occupy and the strength at the coating Steel interface.
Fig. 5 is a graph showing relationship between the developed interfacial area ratio Sdr and the strength of the coating Steel interface.
Fig. 6 is a graph showing, of a steel sheet containing at least one kind of Ti, Nb and V, an influence of a content of Si and a temperature rise speed at a galvannealing process on an area ratio of fine irregularities.
Fig. 7 is a diagram schematically showing a test sample that is used in tensile test for evaluating the coating adhesion 1.
Fig. 8 is a diagram schematically showing a test (bending-unbending test) for evaluating the coating adhesion 2.
Fig. 9 is a diagram schematically showing a test in which for evaluating the coating adhesion 4, a test sample is disposed in a bead die followed by pressing in a horseshoe shape.
Figs. 10A and 10B each are a 3-D SEM image of a surface of the base Steel after the coating layer of the galvannealed steel sheet is removed, Fig. 10A showing a case of a material poor in the adhesion (comparative example), Fig. 10B showing a case of a material excellent in the adhesion (inventive example).

Descriptions of reference numerals in the respective drawings are as follows.
- 1:: irregularity curve
- 2:: base
- 3, 4:: top
- 5:: test sample
- 6:: adhesive
- 7:: spacer
- 8:: arrow mark
- 9:: test sample
- 10:: recessed die
- 11:: projected die
- 12:: arrow mark
- 13:: test sample
- 14:: die
- 15:: wrinkle suppressor
- 16:: bead die
- 17:: punch

### Best Mode for Carrying Out the Invention

In what follows, the present invention will be detailed.

The first invention relates to a galvannealed steel sheet excellent in the coating adhesion, wherein, in an interface between a galvannealed layer and a base steel sheet, an irregularity that has a depth of 10 nm or more at a pitch of 0.5 µm or less is present at least one per 5 µm of a length of the interface.

The present inventors, after an extensive study, found that when a continuous fine irregular portion is formed at an interface between a coating layer and a steel sheet, owing to an anchor effect thereof, the adhesion of an interface between the coating layer and the base steel sheet can be remarkably improved.

Each of Figs. 1 and 2 is a SEM photograph that is taken when a continuous fine irregular portion at an interface between a coating layer and a base steel sheet that is one example of the invention is observed with a scanning electron microscope (SEM). Fig. 1 is a surface SEM photograph observed with a scanning electron microscope when a galvannealed layer is dissolved by applying ultrasonic in an alkaline aqueous solution to be removed and a surface of the base steel sheet at an interface between the coating layer and the base steel sheet is exposed. Fig. 2 is a sectional SEM photograph observed with a scanning electron microscope after a section of a galvannealed steel sheet is polished followed by etching with a 0.1 mass percent nital solution. In the irregular portion, the finer a pitch is, the more preferable, and the deeper a depth thereof is, the more preferable. The present inventors , as a result of study of relationship between the coating adhesion and the irregular state at the coating interface, found that an abundance of the irregularities that have a depth of 10 nm or more and exist with a pitch of 0.5 µm or less greatly correlates with the adhesive strength of the coating layer. In the irregular portion at an interface between the coating layer and the base steel sheet, by observing a section of the coating layer with a scanning electron microscope (SEM) or a transmission electron microscope (TEM), a pitch and a depth can be measured. A measuring method thereof will be shown below.

Measurements of the pitch and the depth are carried out as follows. That is, as shown in Fig. 3, with an irregular curve 1 that is at an interface and can be confirmed by the section observation, in the irregular curve 1, within a certain reference length L (for instance, 0.5 µm), a base 2 that is at a position lowest in height and two tops 3, 4 that are at positions highest in height on each of both sides of the base 2 are found out, a distance in a straight line measured in a length direction between these two tops 3,4 is taken as a pitch P and a distance in a straight line measured in a height direction between, the top 3 which is the lower one of the two tops 3, 4 and the base 2 is taken as a depth D. When with this measurement method a depth D is 10 nm or more in the reference length L (for instance, 0.5 µm), there is a fine irregularity that has a depth D of 10 µm or more at a pitch P of 0.5 µm or less.

However, in the invention, it is necessary that the irregularity having a depth of 10 nm or more at a pitch of 0.5 µm or less exists at least one per 5 µm of a length of interface. (Here, the length of interface means a distance in a straight line between two points on an interface in a cross section in a thickness direction.) This is because unless the irregularity exists at this ratio, it does not contribute to an improvement in the coating adhesion. The measurement of the irregularities is carried out as explained bellow. That is, a cross section of the coating layer having a length of 10 µm is divided into 20 of the reference length L (0.5 µm), 20 viewing fields are observed (Each of the viewing fields is measured at a magnification of at least 5000 times or more.), and, among these, the number of the viewing fields that have the fine irregularity having a depth D of 10 nm or more at a pitch P of 0.5 µm or less is counted. The measurement is repeated 5 times of an arbitrary cross section of the coating layer, and a percentage of the number of the viewing fields that have the fine irregularity to a total number of viewing fields (20 x 5 = 100) is taken as a ratio that the fine irregularities occupy. When the ratio is 10 percent or more, the above condition is considered satisfied.

In Fig. 4, relationship between thus measured ratio that the fine irregularities occupy and the strength at the coating Steel interface is shown. From Fig. 4, it is found that when the ratio that the fine irregularities occupy is 10 percent or more, the strength at the coating steel interface shows a high value. Here, the strength at the coating steel interface is a value obtained by carrying out a tensile test according to a method described in a later example (evaluation of the coating adhesion 1) followed by dividing the tensile strength by an adhered area.

From the above, in the invention, it is necessary that, in an interface between a galvannealed layer and a base steel sheet, an irregularity that has a depth of 10 nm or more at a pitch of 0.5 µm or less exists at least one per 5 µm of a length of the interface.

There is the directionality in the formation of the irregularities as shown in Fig. 1. However, a cross section in a direction where the irregularities exist most densely has only to satisfy the condition.

Further disclosed is a galvannealed steel sheet excellent in the coating adhesion, wherein, as to a surface shape of a base steel sheet observed after a galvannealed layer is removed, a developed interfacial area ratio Sdr measured by use of a high-pass filter with a cut-off wavelength of 0.5 µm is 2.0 percent or more.

The inventors paid attention to a developed interfacial area ratio Sdr as an index that can measure from a surface an extent of a continuous irregularity of interfaces of steel sheets shown in Figs. 1 and 2. The developed interfacial area ratio expresses a ratio of an area of an actually irregular surface to an area where the irregularity does not exist in a measurement region and is a value expressed by the following equation. $Developed interfacial area ratio \left(Sdr\right) = \left(A-B\right) / B \times 100$
A: a surface area of an actually irregular interface in a measurement region
B: an area of a plane where an irregularity does not exist in a measurement region

Accordingly, in an interface where the irregularity is large and a surface area is large, the Sdr takes a large value. A shape of the coating interface is formed of very fine irregularities; accordingly, quantitative evaluation was very difficult. However, it is considered to evaluate the fine irregularity by excellently exposing an interface followed by taking a SEM photograph at a high magnification, and thereby precisely calculating the evaluation index. That is, a surface of a base steel after a coating layer of a galvannealed steel sheet was removed, after coating with several tens nanometers of Au so as not to affect on a surface composition, was measured with an electron beam three-dimensional surface roughness analyzer ERA-8800FE manufactured by Elionics Co. , Ltd. followed by shape analysis, and thereby the developed interfacial area ratio Sdr was obtained. The shape analysis was carried out at an accelerating voltage of 15 kV, a viewing field that was magnified at a magnification of 10000 (viewing field area is 12 µm × 9 µm) was taken in at a resolving power of 1200 × 900 points, followed by data processing. A value of the developed interfacial area ratio Sdr is obtained by measuring an arbitrarily selected area followed by averaging. In the calibration that was performed in a height direction with the device, a SHS thin film step standard (with three steps of 18, 88 and 450 nm) for contact stylus and optical surface roughness analyzer manufactured by VLSI Standard Inc. having traceable performance to the National Institute of Standards and Technology in the U.S. was used. Furthermore, a high pass filter having a cut-off wavelength of 0.5 µm was applied and an obtained value was supplied for calculation of three-dimensional shape parameter. The processing is important to remove an influence of undulation having a long period and thereby to evaluate the irregularities having targeted sizes. The cut-off wavelength as well has to be properly selected to a size of the irregularity that is to be evaluated. After studying variously, results processed with a high pass filter having a cut-off wavelength of 0.5 µm were found excellent in the correlation with the interface strength and in the reproducibility. Accordingly, under this condition, the data processing was carried out. Examples of measurement are shown in Figs. 10A and 10B. Fig. 10A is a 3D-SEM image of a sample poor in the adhesion (comparative example) and Fig. 10B is a 3D-SEM image of a product excellent in the adhesion (inventive example), and values of the developed interfacial area ratio Sdr, respectively, were 1.7 percent for the comparative example and 2. 5 percent for the inventive example. That is, there are distinct differences in the images and the Sdr values. On the other hand, the Ra in each of the images is 0.00531 µm for the comparative example and 0.00547 µm for the inventive example. That is, it is found that according to the Ra that is generally used, the difference cannot be quantified and the effectiveness of the evaluation method can be confirmed.

Fig. 5 is a graph showing relationship between values of the developed interfacial area ratio Sdr and the strengths of the coating interface at the interface between the coating layer and the base steel sheet. From Fig. 5, it is found that in the case of the value of the developed interfacial area ratio Sdr being 2.0 percent or more, high interface strength can be obtained. Herein, a shape is specified with the developed interfacial area ratio of three-dimensional parameter considered most fitted to the evaluation. However, after processing with a similar high pass filter, it can be evaluated with RSm (an average length of roughness curve element) of two-dimensional parameter.

In the next place, a steel sheet suitably used as a base steel sheet in the invention will be explained.

The base steel sheet contains, by mass percent, 0.25 percent or less of C, 0.03 to 2.0 percent of Si and 0.005 to 0.07 percent of P and has a composition satisfying the following equation (1).

Note $\left[C\right] + \left[P\right] \leq \left[Si\right]$

Here, [C], [P] and [Si], respectively, mean contents (mass percent) of C, P and Si in the base steel sheet.

Reasons for components C, P and Si in the base steel sheet (mother material) being in the above ranges are as follows. In what follows, contents (percent) of elements all mean mass percent.

### C: 0.25 percent or less

Since the strength of steel can be easily increased when a content of C is increased, it is indispensable element for increasing the strength of the base steel sheet (mother material). However, since when the content of C is excessive, the ductility or the weldability of the base material is deteriorated, a content of C is set at 0.25 percent or less. Furthermore, in the case of a steel sheet being used for the deep drawing, C desirably is not added as far as possible.

### Si: 0.03 to 2.0 percent

Si is a strengthening element of steel and an element that allows forming a continuous irregular portion at an interface between a coating layer and a base steel sheet. Though a detail is not understood, when a content of Si is less than 0.03 percent, a continuous irregular portion is formed with difficulty. On the other hand, since Si delays an alloying reaction, it is preferable not to add as far as possible from a viewpoint of alloying. Furthermore, when a content of Si exceeds 2.0 percent, an effect of improving the coating adhesion saturates, and a problem in that the alloying reaction is excessively delayed is likely to be caused. Accordingly, a content of Si is in the range of 0.03 to 2.0 percent.

### P: 0.005 to 0.07 percent

P is a strengthening element of steel. However, it is a remarkable grain boundary segregation element, delays the reaction excessively and deteriorates the weldability. Accordingly, it is preferably reduced as far as possible; that is, P is contained 0.07 percent or less. However, in order to reduce a content of P in the steel more than necessary, electrolytic iron high in the purity and grade is necessarily used, resulting in a problem in that economical efficiency is damaged. Accordingly, a content of P is 0.005 percent or more.

In the invention, the contents of C, Si and P in the base steel sheet are limited in the above ranges and satisfy the following equation (1).

Note $\left[C\right] + \left[P\right] \leq \left[Si\right]$

Here, [C], [P] and [Si], respectively, mean contents (mass percent) of C, P and Si in the base steel sheet.

As mentioned above, when Si is added to steel, a continuous irregular portion is formed at an interface between the coating layer and the base steel sheet and thereby the coating adhesion can be greatly improved. However, when, in addition to Si, C and P are added in combination in the steel, a continuous irregular portion is suppressed from forming at an interface between the coating layer and the base steel sheet and thereby an improvement in the coating adhesion is disturbed. As mentioned above, C and P are strengthening elements of steel and indispensable elements for strengthening. That is, in order to form a continuous irregular portion that contributes to the coating adhesion, in accordance with amounts of C and P added, an amount of Si added is necessary to be controlled as shown in the above equation (1). In the case of [C] + [P] ≤ [Si], a continuous irregular portion can be easily formed at an interface between the coating layer and the base steel sheet.

Furthermore, elements other than C, Si and P are contained in the steel.

As the other elements, Mn, S and Al can be cited as components that may be contained in the base steel sheet. Preferable ranges of the elements are as follows.

### Mn: 5 percent or less

Mn is a strengthening element of steel and can be contained as needs arise. However, when a content of Mn exceeds 5 percent, the workability and the economic efficiency of the base material are damaged; accordingly, a content Mn is preferably set at 5 percent or less. In order to obtain sufficient strengthening effect of the steel, Mn is preferably contained 0.5 percent or more.

### S: 0.01 percent or less

S is an element inevitably present in steel. When S is contained more than 0.01 percent, the workability of the base steel sheet tends to deteriorate. Accordingly, a content of S is preferably set at 0.01 percent or less.

### Al: 0.08 percent or less

Al works as a deoxidizing agent and can be added as needs arise. However, when a content of Al exceeds 0.08 percent, its effect only saturates and an increase in the manufacturing cost is invited; accordingly, a content of Al is preferably set at 0.08 percent or less. In order to develop a function as the deoxidizing agent, a content of Al is preferably set at 0.02 percent or more.

As the strengthening element of the steel, at least one kind selected from Ti, Nb and V is contained. All of Ti, Nb and C can bind with C and N in the steel to form a fine precipitate and thereby strengthening the base steel sheet. When each of Ti, Nb and V components is added more than 0.2 percent, there is a tendency of damaging the workability; accordingly, contents of Ti, Nb and V each are set at 0.2 percent or less.

Furthermore, at least one kind selected from Ti, Nb and V, when added in a proper amount, combines with dissolved P to form a fine precipitate, Fe-(Ti, Nb, V)-P, and thereby the dissolved P is partly rendered harmless. As a result, without excessively delaying a mutual diffusion reaction of Fe and Zn, the coating interface strength can be largely improved. In order to develop such an effect, in accordance with an amount of P in the steel, at least one kind of Ti, Nb and V satisfying the following equation (3) is contained. $\left[Ti\right] + \left[Nb\right] + \left[V\right] \geq \left[P\right]$

Here, [Ti], [Nb], [V] and [P], respectively, mean consents (mass percent) of Ti, Nb, V and P.

Components such as Cr, Mo, Cu, Ni, Ca, B, N and Sb other than the abovementioned components in the base steel sheet, since presence thereof does not at all contribute to the effects of the invention, may be added as needs arise. Reasons for addition and preferable ranges thereof are as follows.

### Cr: 0.5 percent or less

This is a strengthening element of steel and can be added as needs arise. However, since the coating properties are deteriorated and the alloying nonuniformity is caused, it is preferably added by 0.5 percent or less.

### Mo: 1.0 percent or less

This is a strengthening element of steel and can be added as needs arise. However, since the alloying delay is caused and the workability and the economic efficiency are damaged, it is preferably added by 1 percent or less.

### Cu: 0.5 percent or less

This is a coating property improving element and can be added as needs arise. However, when it is added more than 0.5 percent, an effect thereof saturates and the economic efficiency is damaged. Accordingly, it is preferably added by 0.5 percent or less.

### Ni: 0.5 percent or less

This is a coating property improving element and can be added as needs arise. However, when it is added more than 0.5 percent, an effect thereof saturates and the economic efficiency is damaged. Accordingly, it is preferably added by 0.5 percent or less.

### Ca: 0.01 percent or less

This works as a deoxidizing agent and may be contained as needs arise. However, when it is added more than 0.01 percent, an effect thereof saturates. Accordingly, an addition of 0.01 percent or less is preferable.

### B: 0.003 percent or less

Owing to grain boundary strengthening, the cold work embrittlement can be improved. However, since an effect thereof saturates at more than 0.003 percent, it is preferably added by 0.003 percent or less.

### N: 0.01 percent or less

N comes in as an impurity. When it exceeds 0.01 percent, the ductility is deteriorated. Accordingly, it is preferably added by 0.01 percent or less.

### Sb: 0.05 percent or less

This is a coating appearance improvement element and can be added as needs arise. However, when it is added more than 0.05 percent, an effect thereof saturates and the economic efficiency is damaged. Accordingly, it is preferably added by 0.05 percent or less.

The balance other than the abovementioned elements is preferably made of Fe and inevitable impurities. Furthermore, in the invention, the tensile strength of the base steel sheet that is measured with a No. 5 test piece stipulated in JIS Z2201 and according to a tensile test method stipulated in JIS G3302 is preferably 440 MPa or more. When the base steel sheet is made a high tension steel sheet having the tensile strength of 440 MPa or more, in the fields of automobiles, home electric appliances, construction materials and so on, demands for higher strength and/or lighter weight base can be satisfied.

In the next place, a manufacturing method of forming an irregularity as defined herein (an irregularity that has a depth of 10 nm or more at a pitch of 0.5 µm or less and is present at least one per 5 µm of a length of the interface or an irregularity that has the developed interfacial area ratio Sdr of 2.0 percent or more when a surface shape of a base steel sheet observed by peeling a galvannealed layer is measured with a high pass filter with a cut-off wavelength of 0.5 µm) at an interface between a galvannealed layer and a base steel sheet will be explained below.

A galvannealed steel sheet according to the invention is manufactured, with a steel sheet having the abovementioned component composition as a base steel sheet, by applying a hot-dip galvanizing process and a subsequent galvannealing process. Here, the base steel sheet may be any one of a hot rolled steel sheet, a cold rolled steel sheet, or a steel sheet obtained by specially heat-treating these and is not restricted to particular one. The base steel sheet, after a surface thereof is cleansed by degreasing and/or by washing with acid in a pre-treatment process, or, by omitting the pre-treatment process, an oil component on a surface of the base steel sheet is burned and removed in a pre-heating furnace, is annealed at a temperature in the range of 750 to 900 degree centigrade in a reducing atmosphere. Thereby, a scale on the surface of the base steel sheet is reduced and a surface state suitable for subsequent hot-dip galvanizing is obtained. Now, in the case of the base steel sheet in which Si is added to steel, even in a reducing atmosphere to Fe, in some cases, Si is selectively surface oxidized, resulting in forming an oxide concentrated on a surface. The silicon oxide oxidized selectively on a surface deteriorates the wettability with molten zinc during the coating to result in causing a bare spots surface. Accordingly, it is necessary to suppress the selective surface oxidation in a reducing atmosphere. Furthermore, as mentioned above, although Si in steel has a function of allowing forming a fine irregular portion at an interface between a coating layer and a base steel sheet, since silicon does not develop an effect when it exists as oxide, it is necessary to substantially suppress the selective surface oxidation in a reducing atmosphere from occurring.

Substantially suppressing the selective surface oxidation of Si from occurring means as mentioned above a state where the coating wettability is lowered and thereby the bare spots is inhibited from occurring; that is, there is no problems as far as it is a state where the bare spots is not caused.

As a method of obtaining a state where, with steel to which Si is added, Si does not substantially undergo the selective surface oxidation in a reducing atmosphere, there is a method in which, prior to annealing in a reducing atmosphere, in a weak acidic atmosphere, a pre-heating or heating process is applied. That is, in a weak acidic atmosphere a surface of the steel sheet is oxidized to form a thin iron scale followed by annealing in a reducing atmosphere to form reduced iron on the surface of the steel sheet, and thereby the selective surface oxidation of Si can be suppressed from occurring. The weak acidic atmosphere is an acidic atmosphere to an extent that allows sufficiently applying reduction in a later reducing atmosphere and not particularly restricted. As a weak acidic atmosphere, an atmosphere where 0.01 to 0.5 volume percent of oxygen is contained, a dew point is in the range of -20 to +20 degree centigrade, the balance is made of nitrogen and a temperature is in the range of 300 to 500 degree centigrade is employed, and as a reducing atmosphere, an atmosphere where 3 to 20 volume percent of hydrogen is contained, the balance is made of nitrogen and a temperature is in the range of 750 to 900 degree centigrade is employed.

When a surface of a steel sheet is oxidized in a weak acidic atmosphere to form a thin iron scale followed by annealing in a reducing atmosphere and thereby reduced iron is formed on a surface of the steel sheet, Fe oxide formed in the weak acidic atmosphere is reduced in an annealing process in the subsequent reducing atmosphere and silicon oxide, without being oxidized even in the annealing process in the reducing atmosphere, remains as internal oxide in base steel immediate below a surface of the base steel sheet. The internal oxide is distinguished from an oxide that is formed according to the selective surface oxidization of Si and works so as to suppress Si from being selectively surface oxidized during the annealing in a reducing atmosphere. The internal oxide remains in a hot-dip galvanizing process and in a subsequent galvannealing process.

The base steel sheet after the annealing is cooled in the reducing atmosphere to a temperature suitable for the coating, preferably in the range of 440 to 540 degree centigrade, dipped without exposing to air in a molten zinc coating bath to apply the coating. At this time, an atmosphere immediately before the coating is made an atmosphere having an oxygen concentration of 0.005 volume percent or less. This is because oxygen, in particular, lowers the reactivity of a surface of the base steel sheet to disturb the formation of a fine irregularity at an interface between a coating layer and the base steel sheet. Residual gases other than oxygen, not particularly affecting on the formation of the fine irregularity, are not limited. For instance, an atmosphere containing 3 to 20 volume percent of hydrogen and the balance of nitrogen can be cited. Furthermore, since oxygen lowers the wettability with molten zinc to induce the bare spots, also from this meaning, it is better to be low.

The hot-dip galvanizing process has only to be conducted according to an existing method. For instance, it is preferable that a temperature of a coating bath is set in the range of substantially 450 to 500 degree centigrade and a concentration of Al in the coating bath is set in the range of 0.10 to 0.15 mass percent. However, depending on components in the steel, the coating conditions mentioned above have to be altered. However, difference of the coating conditions, not bringing about any contribution to the effects of the invention, is not particularly restricted.

As a method of adjusting a thickness of a coating layer after the coating, without being restricted to a particular one, a general gas-wiping is used; that is, a gas pressure of the gas-wiping, a distance between a wiping nozzle and a steel sheet and so on are used to adjust. At this time, a thickness of the coating layer is preferably in the range of 3 to 15 µm. When it is less than 3 µm, the rust resistance cannot be sufficiently obtained. On the other hand, when it exceeds 15 µm, not only an improving effect of the rust resistance saturates but also the workability and the economic efficiency unfavorably tend to be lowered.

A method of galvannealing process after the coating thickness is adjusted can be applied by use of a method such as gas heating or induction heating. However, it is necessary that an average temperature rise speed during heating to a galvannealing temperature is 20 degree centigrade/s or more. This is because in the case of less than 20 degree centigrade/s, a staying time in a low temperature region is long to cause a delay in galvannealing reaction, and thereby a fine irregularity at an interface between a coating layer and a base steel sheet is inhibited from forming.

Furthermore, since Ti, Nb and V are contained in the above range in the base steel sheet, a temperature rise speed during heating in the galvannealing process and a content of Si in the base steel sheet are necessary to satisfy the equation (2) below. $ST \geq 3.25 / \left[Si\right]$

Here, in the equation, ST expresses a temperature rise speed (degree centigrade/s) and [Si] denotes a content (mass percent) of Si in the steel sheet.

According to inventors' research, it was found that when Ti, Nb and V are contained in steel, in the case of a content of Si being low, even when a temperature rise speed in the galvannealing process is set at 20 degree centigrade/s or more, in some cases, an inventive fine irregularity in an interface between the coating layer and the base steel sheet is not formed; that is, a temperature rise speed is necessary to raise in accordance with the content of Si.

Fig. 6 is a graph showing, of steel sheets that contain at least one kind of Ti, Nb and V in a range that satisfies the equation (3), influence of a content of Si and a temperature rise speed on a an area ratio of fine irregularity. It is found that when the equation (2) is satisfied, the area ratio of the fine irregularity becomes 10 percent or more.

Although a time of galvannealing is not particularly restricted, a content of Fe in the coating layer is preferably controlled in the range of 8 to 13 mass percent. When the content of Fe in the coating layer is less than 8 mass percent, since the aforementioned Fe-Zn alloy phase is not sufficiently formed and a soft η-Zn phase remains on a surface of the coating layer, in some cases, the workability and the adhesion are damaged. On the other hand, when the content of Fe in the coating layer exceeds 13 mass percent, there is a problem in that a hard and brittle Fe-Zn alloy phase (for instance, a Γ phase or a Γ1 phase) is formed excessively thick in an interface between the coating layer and the base steel sheet, and thereby the embrittlement in the interface between the coating layer and the steel sheet is forwarded.

"A content of Fe in a coating layer" here denotes a mass percentage of Fe in a coating layer to an entire coating layer, that is, an average content of Fe. A method of measuring a content of Fe in the coating layer is carried out in such manner that for instance, a galvannealed layer is dissolved with hydrochloric acid added with an inhibitor followed by measuring by ICP (Inductively Coupled Plasma) emission spectrometry.

A method of controlling a content of Fe in the coating layer in the range of 8 to 13 mass percent is not restricted to particular one. In general, it is controlled through a sheet temperature and a staying time in a galvannealing heating furnace and so on. The staying time in the furnace is preferably shorter from a viewpoint of the productivity and specifically operated within substantially 5 to 30 sec. Furthermore, the sheet temperature, though being selected depending on the staying time in the furnace, is generally operated in the range of 460 to 600 degree centigrade. In the case of less than 460 degree centigrade, in order to control the content of Fe in the coating layer in the range of 8 to 13 mass percent, a long galvannealing process is forced to operate; accordingly, it becomes necessary to make a speed of steel sheet extremely slow or to use a very long galvannealing furnace. As a result, since there is a problem in that the productivity is lowered or huge equipment expense is necessary, it is preferably operated at 460 degree centigrade or more. On the other hand, when it exceeds 600 degree centigrade, there is a problem in that in an interface between the coating layer and the base steel sheet, a hard and brittle Fe-Zn alloy phase (for instance, a Γ phase or a Γ1 phase) tends to be formed excessively thick, and thereby the embrittlement of the interface between the coating layer and the base steel sheet is enhanced. Accordingly, it is preferably operated at 600 degree centigrade or less.

After the galvannealing process, cooling is immediately followed. A method of cooling, though not particularly restricted, is desirably applied by quenching at 30 degree centigrade/s or more to 420 degree centigrade where the galvannealing reaction comes to completion, for instance, an existing method such as gas cooling and mist cooling has only to be applied.

In what was mentioned above, only one example of embodiments of the invention is shown and the invention can be variously modified in the range of claims.

### Example 1 (not according to the invention)

Each of steel ingots having a chemical composition shown in Table 1 was heated to 1250 degree centigrade to apply hot rolling followed by removing a scale on a surface, and thereby a hot rolled steel sheet having a thickness of 2.0 mm was prepared. Subsequently, cold rolling at the reduction rate of 50 percent was applied to form a cold rolled steel sheet having a thickness of 1.0 mm, followed by cutting out into a width of 70 mm and a length of 180 mm. This was subjected to primary heating at 830 degree centigrade in a heating furnace in a nitrogen atmosphere that contains 3 volume percent of hydrogen and has a dew point of -30 degree centigrade to cleanse a surface thereof, and thereby a base steel sheet was prepared. After the base steel sheet was dipped in 5 percent hydrochloric acid at 60 degree centigrade for 10 sec to apply pickling, recrystallization annealing and hot-dip galvanizing (hereinafter, simply referred to as "galvanizing") were applied by use of a laboratory galvanizing simulator. Conditions for the recrystallization annealing and the galvanizing were as follows.

**(Table 1)**

| Steel No. | The balance of steel composition (mass %) is Fe and inevitable impurities | | | | | | Note |
|---|---|---|---|---|---|---|---|
| | C | Si | Mn | P | sol.Al | S | |
| 1A | 0.03 | 0.1 | 2.2 | 0.065 | 0.03 | 0.003 | |
| 1B | 0.08 | 0.1 | 0.5 | 0.01 | 0.029 | 0.003 | |
| 1C | 0.08 | 0.25 | 2 | 0.01 | 0.042 | 0.003 | |
| 1D | 0.08 | 0.2 | 2.6 | 0.015 | 0.035 | 0.003 | |
| 1E | 0.03 | 0.6 | 2 | 0.01 | 0.05 | 0.003 | |
| 1F | 0.08 | 0.2 | 2 | 0.01 | 0.041 | 0.003 | |
| 1G | 0.08 | 0.6 | 1.95 | 0.01 | 0.045 | 0.003 | Example * |
| 1H | 0.15 | 0.8 | 2.6 | 0.012 | 0.065 | 0.003 | |
| 1I | 0.1 | 0.25 | 2 | 0.015 | 0.029 | 0.003 | |
| 1J | 0.03 | 0.25 | 1.6 | 0.03 | 0.033 | 0.003 | |
| 1K | 0.16 | 0.2 | 0.8 | 0.01 | 0.041 | 0.003 | |
| 1L | 0.25 | 0.3 | 0.8 | 0.012 | 0.041 | 0.003 | |
| 1M | 0.03 | 0.5 | 1.5 | 0.02 | 0.036 | 0.003 | |
| 1N | 0.003 | 0.02 | 0.28 | 0.02 | 0.031 | 0.003 | |
| 1O | 0.002 | 0.02 | 0.09 | 0.014 | 0.04 | 0.003 | |
| 1P | 0.15 | 0.05 | 1.2 | 0.012 | 0.039 | 0.003 | |
| 1Q | 0.15 | 0.1 | 1.2 | 0.012 | 1.5 | 0.003 | |
| 1R | 0.05 | 0.02 | 0.8 | 0.008 | 0.055 | 0.003 | |
| 1S | 0.018 | 0.02 | 0.18 | 0.01 | 0.033 | 0.003 | Comparative Example |
| 1T | 0.01 | 0.1 | 1 | 0.075 | 0.035 | 0.003 | |
| 1U | 0.004 | 0.02 | 0.14 | 0.021 | 0.045 | 0.003 | |
| 1V | 0.08 | 0.07 | 2 | 0.01 | 0.06 | 0.003 | |
| 1W | 0.002 | 0.02 | 0.3 | 0.035 | 0.033 | 0.003 | |
| 1X | 0.12 | 0.1 | 3 | 0.015 | 1.5 | 0.003 | |
| 1Y | 0.08 | 0.05 | 1.5 | 0.03 | 0.041 | 0.003 | |

| | | | | | | | |
|---|---|---|---|---|---|---|---|
| * (not according to the invention) | | | | | | | |

### <Recrystallization annealing>

Atmosphere: 5 volume percent hydrogen + nitrogen (dew point: -35 degree centigrade)
Temperature: 750 degree centigrade
Holding time: 20 sec

### <Coating conditions>

Bath composition: Zn + 0.14 mass percent Al (Fe saturation)
Bath temperature: 460 degree centigrade
Sheet temperature at the time of coating: 460 degree centigrade
Coating time: 1 sec Concentration of oxygen in an atmosphere immediately before
the coating: conditions described in Table 2 (the balance 5 volume percent hydrogen + nitrogen (dew point: -35 degree centigrade))

Obtained coating steel sheets contained 0.2 to 0.5 mass percent of Al and 0.5 to 2 mass percent of Fe in the coating layers. After the coating process above, a galvannealing process was applied in air in an electric heater. Temperature rise speeds and galvannealing temperatures in the galvannealing process were the conditions described in Table 2.

Of each of obtained coating steel sheets, a cooling atmosphere from the recrystallization annealing to the coating, a thickness of a coating layer, a temperature rise speed, a temperature and a holding time in the galvannealing process, a content of Fe in the coating layer, a ratio of fine irregularity formed in an interface between the coating layer and a base steel sheet and a developed interfacial area ratio Sdr are shown in Table 2. Furthermore, a method of evaluating the coating adhesion 1 of the obtained coating steel sheet is shown below and evaluation results are shown together in Table 2.

### <Ratio of interfacial irregularity>

A cross section of an interface of the coating layer and the steel sheet in the obtained steel sheet was observed with a SEM (TEM was used together) over a length of 10 µm in five viewing fields in an arbitrary cross section and a ratio at which fine irregularity (having a depth of 10 nm or more at a pitch of 0.5 µm or less) occupies in an entire coating cross section is taken as an interfacial irregularity ratio (%).

### <Developed interfacial area ratio Sdr>

The coating layer was removed by subjecting to constant-potential electrolysis in an alkaline solution containing NaOH, NaCl, and triethanolamine and thereby an interface between the coating layer and the base steel sheet was exposed. The exposed surface was measured of a surface shape by use of an electron beam three-dimensional surface roughness analyzer ERA-8800FE (manufactured by Elionics Co., Ltd.). A test sample, in order to avoid an influence of a composition of surface, was coated with Au with a thickness of several tens nanometers and supplied for measurement. The shape analysis measurement was performed at an acceleration voltage of 15 kV, a viewing field magnified by 10000 times (viewing field area is 12 µm × 9 µm) was collected at the resolving power of 1200 × 900 points, followed by data processing. A value of the developed interfacial area ratio Sdr was obtained by averaging results obtained by measuring arbitrarily selected three areas. In the calibration that was performed in a height direction with the device, a SHS thin film step standard (with three steps of 18, 88 and 450 nm) for contact stylus and optical surface roughness analyzer manufactured by VLSI Standard Inc. having traceable performance to the NIST that is National Institute of Standard and Technology in the U.S. was used. Furthermore, a high pass filter having a cut-off wavelength of 0.5 µm was applied to supply for calculation of three-dimensional shape parameter.

### <Thickness of coating layer>

A cross section of the obtained coating steel sheet was observed with an optical microscope (magnification: 400 times), a thickness of the coating layer was measured at arbitrary three points , followed by averaging these, and an averaged value was taken as a thickness of the coating layer (µm).

### <Content of Fe in the coating layer>

The coating layer of the obtained coating steel sheet was dissolved with hydrochloric acid added with an inhibitor and Zn and Fe in the coating layer were quantitatively analyzed by ICP emission spectrometry. A mass percentage (mass percent) of Fe to (Zn + Fe) was taken as a content of Fe in the coating layer.

### (Evaluation of the coating adhesion 1)

From the obtained coating steel sheet, two test pieces having a width of 25 mm and a length of 80 mm were cut out, after dipping in a rust preventive oil: 550KH (manufactured by Nihon Parkerizing Co., Ltd.), were left in air standing obliquely for 24 hr, and thus obtained ones were supplied as test samples. As shown in Fig. 7, after an adhesive 6 was coated on surface portions that are adhered of test samples 5, the test samples were stacked so that a length of an overlapped portion X may be 20 mm. As the adhesive 6, E-56 (manufactured by Sunrise MSI Co.,) was used, and by use of spacers 7 (SUS304 wire having a diameter of 0.15 mm) a thickness of the adhesive was maintained constant for each of the test pieces. After the adhesive was coated, heat treatment was applied at 170 degree centigrade for 20 min in a drying oven, thereafter tensile test applying tension in directions of arrow marks 8 was applied by use of an autograph (manufactured by Shimadzu Corporation), and thereby the tensile shear strength and peeling mode were measured, followed by evaluating according to criteria below. The tensile shear strength was evaluated with a ratio (%) to the strength obtained when with a cold rolled steel sheet (non-coating material) having the same steel composition and the same size the tensile test was applied.

### <Evaluation criteria of tensile shear strength>

○○: very good (strength ratio: exceeding 90 %)
○: good (strength ratio: exceeding 80 % and 90 % or less)
Δ: fair (strength ratio: exceeding 60 % and 80 % or less) and
×: bad (strength ratio: 60 % or less)

### <Evaluation criteria of peeling mode>

○○: very good (coagulation peeling in the adhesive)
Δ: fair (partially peeling at an interface of coating layer/base steel sheet)
×: bad (overall peeling at an interface of coating layer/base steel sheet)

In the evaluation criteria of the peeling mode, the peeling at an interface of coating layer/base steel sheet means the peeling at an interface of the coating layer and the base steel sheet. However, depending on the peeling mode, in some cases, the peeling at an interface of the coating layer and the base steel sheet does not occur uniformly, accordingly cases where the peeling occurs within 2 µm on a side of the coating layer or on a side of the base steel sheet from the interface of the coating layer and the base steel sheet are included.

**(Table 2-1)**

| Test sample No. | Steel No. | Concentration of oxygen in a cooling atmosphere until the coating after the recrystallization annealing (vol.%) | Galvannealing condition | | | Galvannealed steel sheet | | | | Evaluation result | | Note |
|---|---|---|---|---|---|---|---|---|---|---|---|---|
| | | | | | | Coating layer | | Base steel sheet | Ratio of fine irregularity in an interface (%) | Coating adhesion 1 | | |
| | | | Temperature rise speed (^{°}C/s) | Galvannealing temperature (°C) | Holding time (s) | Thickness (µm) | Content of Fe (mass %) | Developed interfacial area ratio Sdr (%) | | Tensile shear strength | Peeling mode | |
| 1 | 1A | 0.002 | 25 | 490 | 15 | 7 | 10.8 | 2.2 | 15 | ○ | ○○ | |
| 2 | 1B | 0.002 | 20 | 480 | 10 | 6 | 9.2 | 2.1 | 15 | ○○ | ○○ | |
| 3 | 1C | 0.001 | 25 | 490 | 9 | 3 | 10.3 | 2.5 | 50 | ○○ | ○○ | |
| 4 | 1C | 0.002 | 25 | 490 | 15 | 7 | 9.9 | 2.5 | 45 | ○○ | ○○ | |
| 5 | 1C | 0.002 | 25 | 490 | 22 | 6 | 12.5 | 2.8 | 75 | ○○ | ○○ | |
| 6 | 1C | 0.003 | 30 | 510 | 20 | 14 | 11.2 | 2.6 | 60 | ○○ | ○○ | |
| 7 | 1D | 0.002 | 25 | 500 | 16 | 9 | 11.8 | 2.6 | 55 | ○○ | ○○ | Example* |
| 8 | 1E | 0.002 | 35 | 520 | 20 | 8 | 10.6 | 2.6 | 65 | ○○ | ○○ | |
| 9 | 1F | 0.002 | 25 | 490 | 15 | 10 | 11.0 | 2.3 | 30 | ○○ | ○○ | |
| 10 | 1G | 0.002 | 30 | 520 | 15 | 6 | 11.3 | 2.5 | 50 | ○○ | ○○ | |
| 11 | 1H | 0.004 | 30 | 520 | 20 | 6 | 10.6 | 2.3 | 25 | ○○ | ○○ | |
| 12 | 1I | 0.002 | 20 | 460 | 12 | 4 | 9.1 | 2.1 | 10 | ○ | ○○ | |
| 13 | 1J | 0.002 | 25 | 490 | 20 | 7 | 10.6 | 2.8 | 70 | ○○ | ○○ | |
| 14 | 1K | 0.002 | 30 | 510 | 15 | 6 | 11.2 | 2.8 | 75 | ○○ | ○○ | Example* |
| 15 | 1L | 0.004 | 25 | 480 | 18 | 8 | 11.0 | 2.8 | 65 | ○○ | ○○ | |
| 16 | 1M | 0.002 | 35 | 540 | 6 | 5 | 9.2 | 2.8 | 70 | ○○ | ○○ | |
| 17 | 1N | 0.003 | 20 | 520 | 8 | 7 | 10.0 | 1.6 | 0 | × | Δ | |
| 18 | 1O | 0.002 | 30 | 470 | 15 | 10 | 9.5 | 1.5 | 0 | × | × | |
| 19 | 1P | 0.002 | 20 | 500 | 20 | 6 | 12.3 | 1.7 | 0 | Δ | × | |
| 20 | 1Q | 0.002 | 20 | 490 | 15 | 6 | 10.0 | 1.9 | 0 | Δ | Δ | |
| 21 | 1R | 0.002 | 35 | 490 | 7 | 7 | 8.2 | 1.8 | 0 | Δ | Δ | |
| 22 | 1S | 0.003 | 20 | 520 | 15 | 8 | 12.8 | 1.4 | 0 | × | × | Comparative Example |
| 23 | 1T | 0.002 | 20 | 520 | 22 | 9 | 11.5 | 1.7 | 0 | × | Δ | |
| 24 | 1U | 0.002 | 20 | 510 | 12 | 10 | 11.5 | 1.6 | 0 | × | × | |
| 25 | 1V | 0.001 | 20 | 500 | 9 | 8 | 9.9 | 1.8 | 0 | × | Δ | |
| 26 | 1W | 0.002 | 30 | 490 | 12 | 10 | 9.6 | 1.9 | 0 | Δ | Δ | |
| 27 | 1X | 0.002 | 20 | 520 | 15 | 11 | 11.6 | 1.7 | 0 | × | × | |
| 28 | 1Y | 0.002 | 20 | 470 | 18 | 9 | 11.1 | 1.7 | 0 | Δ | Δ | |
| 29 | 1B | 0.007 | 20 | 480 | 10 | 6 | 9.2 | 1.9 | 5 | Δ | Δ | |

| | | | | | | | | | | | | |
|---|---|---|---|---|---|---|---|---|---|---|---|---|
| * (not according to the invention) | | | | | | | | | | | | |

From the evaluation results shown in Table 2, it is found that galvannealed steel sheets of the examples, in comparison with existing steel sheets (comparative examples), are largely heightened in the strength of the interface between the coating layer and the base steel sheet and improved in the coating adhesion thereof.

### Example 2

Each of steel ingots having a chemical composition shown in Table 3 was heated at 1250 degree centigrade to apply the hot rolling followed by removing a scale on a surface, and thereby a hot rolled steel sheet having a thickness of 2.0 mm was prepared. Subsequently, the cold rolling at the reduction rate of 50 percent was applied to form a cold rolled steel sheet having a thickness of 1.0 mm, followed by cutting out into a width of 70 mm and a length of 180 mm, further followed by surface cleaning, and thereby a base steel sheet was obtained. The base steel sheet was dipped in 5 percent hydrochloric acid at 60 degree centigrade for 10 sec to apply pickling, thereafter, subjected to primary heating by holding at 400 degree centigrade for 1 sec in a nitrogen atmosphere (dew point: + 20 degree centigrade) containing 0.1 volume percent of oxygen, and thereafter subjected to a secondary heating by holding at 750 degree centigrade for 1 sec in a nitrogen atmosphere (dew point: + 20 degree centigrade) containing 5 volume percent of hydrogen. To the heat treated base steel sheet, recrystallization annealing and coating were applied by use of a laboratory galvanizing simulator. Conditions for the recrystallization annealing and the coating were as follows.

**(Table 3)**

| Steel No. | The balance of steel composition (mass %) is Fe and inevitable impurities | | | | | | | 3.25/Si | Note |
|---|---|---|---|---|---|---|---|---|---|
| | C | Si | Mn | P | Ti | Nb | V | | |
| 2A | 0.025 | 0.13 | 2 | 0.03 | 0.02 | 0,01 | 0.01 | 25 | |
| 2B | 0,08 | 0.1 | 0.5 | 0.01 | 0.02 | 0.01 | - | 33 | |
| 2C | 0.08 | 0.25 | 2 | 0.01 | 0.02 | 0.06 | - | 13 | |
| 2D | 0.08 | 0.2 | 2.6 | 0.015 | 0.02 | 0.05 | - | 16 | |
| 2E | 0.075 | 0.6 | 2 | 0.01 | - | 0.03 | - | 5 | |
| 2F | 0.08 | 0.2 | 2 | 0.01 | 0.02 | - | - | 16 | |
| 2G | 0.08 | 0.6 | 1.95 | 0.01 | 0.01 | 0.01 | - | 5 | Example |
| 2H | 0.15 | 0.8 | 2.6 | 0.012 | 0.01 | 0.01 | - | 4 | |
| 2I | 0.1 | 0.3 | 2 | 0.015 | - | 0.02 | 0.02 | 11 | |
| 2J | 0.08 | 0.25 | 1.6 | 0.03 | - | 0.025 | 0.05 | 13 | |
| 2K | 0.16 | 0.2 | 0.8 | 0.01 | 0.01 | 0.01 | - | 16 | |
| 2L | 0.25 | 0.3 | 0.8 | 0.012 | 0.02 | 0.03 | - | 11 | |
| 2M | 0.04 | 0.16 | 3 | 0.04 | 0.02 | 0.03 | 0.01 | 20 | |
| 2N | 0.003 | 0.02 | 0.28 | 0.02 | 0.02 | 0.01 | - | 163 | |
| 2O | 0.002 | 0.02 | 0.09 | 0.014 | 0.02 | 0.01 | - | 163 | |
| 2P | 0.15 | 0.1 | 1.2 | 0.012 | 0.01 | - | - | 33 | |
| 2Q | 0.15 | 0.02 | 1.2 | 0.012 | 0.02 | 0.01 | 0.01 | 163 | |
| 2R | 0.05 | 0.02 | 0.8 | 0.008 | 0.02 | 0.05 | - | 163 | |
| 2S | 0.018 | 0.02 | 0.18 | 0.01 | 0.02 | 0.01 | - | 163 | Comparative Example |
| 2T | 0.01 | 0.12 | 1 | 0.075 | 0.02 | 0.05 | - | 27 | |
| 2U | 0.004 | 0.03 | 0.14 | 0.04 | 0.01 | 0.01 | - | 108 | |
| 2V | 0.08 | 0.07 | 2 | 0.01 | 0.02 | 0.01 | - | 46 | |
| 2W | 0.002 | 0.02 | 0.1 | 0.01 | 0.01 | 0.01 | - | 163 | |
| 2X | 0.002 | 0.03 | 0.3 | 0.035 | 0.02 | 0.01 | 0.02 | 108 | |
| 2Y | 0.12 | 0.02 | 1.5 | 0.015 | 0.02 | 0.01 | - | 163 | |
| 2Z | 0.08 | 0.05 | 1.5 | 0.03 | 0.02 | 0.03 | - | 65 | |

### <Recrystallization annealing>

Atmosphere: 5 volume percent hydrogen + nitrogen (dew point: -35 degree centigrade)
Temperature: 830 degree centigrade
Holding time: 20 sec

### <coating condition>

Bath composition: Zn + 0.13 mass percent Al (Fe saturation)
Bath temperature: 460 degree centigrade
Sheet temperature at the time of coating: 460 degree centigrade
Coating time: 1 sec Concentration of oxygen in an atmosphere immediately before
the coating: conditions described in Table 4 (the balance 5 volume percent hydrogen + nitrogen (dew point: -35 degree centigrade))

Obtained coating steel sheets contained 0.2 to 0.5 mass percent of Al and 0.5 to 2 mass percent of Fe in the coating layer. After the coating process, the galvannealing process was applied in air in an electric heather. The temperature rise speeds and galvannealing temperatures in the galvannealing process were the conditions described in Table 4.

Of each of obtained coating steel sheets, a cooling atmosphere from the recrystallization annealing to the coating, a thickness of a coating layer, a temperature rise speed, a temperature and a holding time in the galvannealing process, a content of Fe in the coating layer, a ratio of fine irregularity formed in an interface between the coating layer and a base steel sheet and a developed interfacial area ratio Sdr were investigated similarly to a method explained in the example 1. Furthermore, in addition to the evaluation of the abovementioned coating adhesion 1, evaluation of the coating adhesion 2 shown below was carried out. Results of these are shown in Table 4. furthermore, a method of evaluating the coating adhesion of the obtained coating steel sheet is shown below and evaluation results are shown together in Table 4.

### (Evaluation of the coating adhesion 2)

From each of the obtained steel sheets, a test piece having a width of 20 mm and a length of 180 mm was cut out followed by removing burrs, after dipping in rust-preventive oil 550KH (manufactured by Nihon Parkerizing Co. , Ltd.), left in air for 24 hr while standing obliquely, and thus obtained one was used as a test sample. A test sample 9 was disposed on a recessed die 10 such as shown in Fig. 8, and a test in which a bending and unbending operation is applied by lowering a projected die 11 and thereby indenting a surface of the test sample 9 with a load W was carried out. A surface of the die was polished with #1200 polishing paper and cleaning of accretions was carried out each time. An indentation load P of the die was set at 8 kN and the drawing speed of the test sample was set at 20 mm/s. After the test, the test sample was slightly degreased, followed by adhering a cellophane tape (width: 24 mm, manufactured by Nichiban Corp.) to a sliding portion with the die. An amount of Zn adhered to the cellophane tape when it was peeled was measured as the number of counts by X-ray fluorescence analysis, and evaluation was carried out according to the following criteria.

### <Evaluation criteria of the coating adhesion 2>

○○: Very good (number of counts: 25 or less)
○: good (number of counts: more than 25 and 50 or less)
Δ: fair (number of counts: more than 50 and 150 or less)
×: bad (number of counts: more than 150)

**(Table 4-1)**

| Test sample No. | Steel No. | Concentration of oxygen in a cooling atmosphere until the coating after the recrystallization annealing (vol.%) | Alloying condition | | | Galvannealed steel sheet | | | | Evaluation result | | | Note |
|---|---|---|---|---|---|---|---|---|---|---|---|---|---|
| | | | | | | Coating layer | | Base steel sheet | Ratio of fine irregularity in an interface (%) | Coating adhesion 1 | | Coating adhesion 2 | |
| | | | Temperature rise speed (°C/s) | Alloying temperature (°C) | Holding time (s) | Thickness (µm) | Content of Fe (mass %) | Developed interfacial area ratio Sdr (%) | | Tensile shear strength | Peeling mode | | |
| 1 | 2A | 0.001 | 30 | 520 | 15 | 6 | 10.5 | 2.6 | 60 | ○ | ○○ | ○○ | Example |
| 2 | 2B | 0.002 | 35 | 480 | 12 | 7 | 9.5 | 2.6 | 50 | ○○ | ○○ | ○○ | |
| 3 | 2C | 0.001 | 25 | 490 | 10 | 3 | 10.5 | 2.6 | 55 | ○○ | ○○ | ○○ | |
| 4 | 2C | 0.001 | 25 | 490 | 15 | 7 | 9.9 | 2.5 | 50 | ○○ | ○○ | ○○ | |
| 5 | 2C | 0.002 | 25 | 490 | 25 | 6 | 12.8 | 2.8 | 70 | ○○ | ○○ | ○ | |
| 6 | 2C | 0.002 | 25 | 520 | 25 | 14 | 11.0 | 2.7 | 65 | ○○ | ○○ | ○○ | |
| 7 | 2D | 0.002 | 25 | 500 | 15 | 9 | 11.6 | 2.6 | 50 | ○○ | ○○ | ○○ | |
| 8 | 2E | 0.003 | 25 | 520 | 17 | 8 | 10.4 | 2.5 | 50 | ○○ | ○○ | ○○ | |
| 9 | 2F | 0.002 | 25 | 490 | 15 | 11 | 11.2 | 2.6 | 60 | ○○ | ○○ | ○○ | |
| 10 | 2G | 0.002 | 25 | 500 | 20 | 6 | 10.9 | 2.6 | 50 | ○○ | ○○ | ○○ | |
| 11 | 2H | 0.004 | 25 | 520 | 15 | 6 | 9.9 | 2.5 | 45 | ○○ | ○○ | ○○ | |
| 12 | 2I | 0.002 | 25 | 460 | 8 | 4 | 8.9 | 2.1 | 15 | ○ | ○○ | ○○ | |
| 13 | 2J | 0.001 | 25 | 490 | 20 | 7 | 10.6 | 2.5 | 50 | ○○ | ○○ | ○○ | |
| 14 | 2K | 0.002 | 25 | 460 | 30 | 7 | 11.2 | 2.6 | 60 | ○○ | ○○ | ○○ | |
| 15 | 2L | 0.002 | 25 | 480 | 20 | 8 | 11.1 | 2.5 | 55 | ○○ | ○○ | ○○ | Example |
| 16 | 2M | 0.002 | 25 | 560 | 5 | 6 | 9.2 | 2.1 | 25 | ○○ | ○○ | ○○ | |
| 17 | 2N | 0.002 | 10 | 520 | 8 | 9 | 10.0 | 1.9 | 8 | Δ | Δ | ○○ | |
| 18 | 2O | 0.002 | 35 | 530 | 5 | 5 | 9.6 | 1.6 | 0 | Δ | Δ | ○○ | |
| 19 | 2P | 0.002 | 15 | 490 | 12 | 6 | 10.0 | 1.9 | 7 | Δ | × | ○○ | |
| 20 | 2Q | 0.003 | 25 | 490 | 8 | 6 | 9.0 | 1.5 | 0 | Δ | A | ○○ | |
| 21 | 2R | 0.002 | 25 | 490 | 7 | 7 | 8.2 | 1.6 | 0 | Δ | Δ | ○ | |
| 22 | 2S | 0.002 | 25 | 500 | 15 | 6 | 12.4 | 1.7 | 3 | × | × | × | Compar ative Example |
| 23 | 2T | 0.002 | 25 | 480 | 18 | 7 | 11.2 | 1.8 | 8 | × | Δ | ○ | |
| 24 | 2U | 0.002 | 25 | 510 | 8 | 9 | 10.4 | 1.6 | 0 | × | × | Δ | |
| 25 | 2V | 0.002 | 25 | 500 | 9 | 8 | 9.9 | 1.7 | 6 | Δ | Δ | ○○ | |
| 26 | 2W | 0.002 | 25 | 490 | 15 | 7 | 10.3 | 1.9 | 9 | Δ | ○ | Δ | |
| 27 | 2X | 0.002 | 25 | 520 | 7 | 10 | 9.5 | 1.8 | 5 | Δ | Δ | ○○ | |
| 28 | 2Y | 0.002 | 25 | 480 | 15 | 8 | 10.5 | 1.4 | 0 | × | × | Δ | |
| 29 | 2Z | 0.002 | 25 | 470 | 18 | 9 | 11.1 | 1.6 | 2 | Δ | Δ | × | |
| 30 | 2B | 0.010 | 35 | 480 | 12 | 7 | 9.5 | 1.9 | 5 | Δ | Δ | Δ | |

From the evaluation results shown in Table 4, it is found that galvannealed steel sheets according to the invention (examples), in comparison with existing steel sheets (comparative examples), are largely heightened in the interfacial strength between the coating layer and the base steel sheet and improved in the coating adhesion.

### Example 3 (not according to the invention)

Each of steel ingots having a chemical composition shown in Table 5 was heated at 1250 degree centigrade to apply hot rolling followed by removing a black skin on a surface, and thereby a hot rolled steel sheet having a thickness of 2.0 mm was prepared. Subsequently, cold rolling at the reduction rate of 65 percent was applied to form a cold rolled steel sheet having a thickness of 0.7 mm, followed by cutting out into a width of 70 mm and a length of 180 mm, further followed by applying a primary heating at 830 degree centigrade in a heating furnace in a nitrogen atmosphere that has a dew point of -30 degree centigrade and contains 3 volume percent of hydrogen to apply surface cleaning, and thereby a base steel sheet was obtained. The base steel sheet was dipped in 5 percent hydrochloric acid at 60 degree centigrade for 10 sec to apply pickling. Thereafter, recrystallization annealing and coating were applied by use of a laboratory galvanizing simulator. Conditions for the recrystallization annealing and the coating are as follows.

**(Table 5)**

| Steel No. | The balance of steel composition (mass %) is Fe and inevitable impurities | | | | Others | Note |
|---|---|---|---|---|---|---|
| | C | Si | Mn | P | | |
| 3A | 0.002 | 0.1 | 1.5 | 0.02 | - | |
| 3B | 0.01 | 0.3 | 1 | 0.07 | - | |
| 3C | 0.007 | 0.1 | 2.2 | 0.05 | - | |
| 3D | 0.03 | 0.06 | 2 | 0.01 | Cu:0.2, Ni:0.1 | |
| 3E | 0.002 | 0.5 | 1.5 | 0.07 | - | |
| 3F | 0.08 | 0.1 | 2 | 0.01 | Cr: 0.05 | |
| 3G | 0.05 | 0.3 | 0.5 | 0.06 | Mo: 0.15 | Example* |
| 3H | 0.15 | 0.3 | 0.7 | 0.02 | - | |
| 3I | 0.1 | 0.25 | 2.6 | 0.06 | Ca: 0.005 | |
| 3J | 0.003 | 0.25 | 2 | 0.01 | B: 0.001 | |
| 3K | 0.16 | 0.3 | 0.8 | 0.01 | - | |
| 3L | 0.25 | 0.5 | 2 | 0.012 | Mo: 0.3, B: 0.002, Ti: 0.02 | |
| 3M | 0.04 | 0.07 | 3 | 0.01 | Sb: 0.01 | |
| 3N | 0.003 | 0.02 | 0.56 | 0.01 | - | |
| 3O | 0.003 | 0.04 | 0.34 | 0.065 | B: 0.002 | |
| 3P | 0.003 | 0.03 | 0.5 | 0.04 | - | |
| 3Q | 0.002 | 0.02 | 0.5 | 0.04 | - | |
| 3R | 0.008 | 0.05 | 0.75 | 0.09 | - | |
| 3S | 0.08 | 0.05 | 2 | 0.01 | Cr: 0.05 | Comparative Example |
| 3T | 0.008 | 0.09 | 1 | 0.09 | - | |
| 3U | 0.004 | 0.02 | 0.14 | 0.021 | - | |
| 3V | 0.08 | 0.07 | 2 | 0.01 | Ca: 0.005 | |
| 3W | 0.002 | 0.01 | 0.1 | 0.01 | Mo: 0.15 | |
| 3X | 0.01 | 0.02 | 0.45 | 0.01 | - | |
| 3Y | 0.12 | 0.02 | 1.5 | 0.015 | - | |
| 3Z | 0.08 | 0.06 | 1.5 | 0.03 | Sb:0.01 | |

| | | | | | | |
|---|---|---|---|---|---|---|
| * (not according to the invention) | | | | | | |

### <Recrystallization annealing>

Atmosphere: 5 volume percent hydrogen + nitrogen (dew point: -35 degree centigrade)
Temperature: 750 degree centigrade
Holding time: 20 sec

### <Coating condition>

Bath composition: Zn + 0.14 mass percent Al (Fe saturation)
Bath temperature: 460 degree centigrade
Sheet temperature at the time of coating: 460 degree centigrade Coating time: 1 sec Concentration of oxygen in an atmosphere immediately before
the coating: conditions described in Table 6 (the balance 5 volume percent hydrogen + nitrogen (dew point: -35 degree centigrade))

Obtained coating steel sheets contained 0.2 to 0.5 mass percent of Al and 0.5 to 2 mass percent of Fe in the coating layers. After the coating process, the galvannealing process was applied in air in an electric heated. The temperature rise speeds and galvannealing temperatures in the galvannealing process were the conditions described in Table 6.

Of each of obtained coating steel sheets, a cooling atmosphere from the recrystallization annealing to the coating, a thickness of a coating layer, a temperature rise speed, a temperature and a holding time in the galvannealing process, a content of Fe in the coating layer, a ratio of fine irregularity formed in an interface between the coating layer and a base steel sheet and a developed interfacial area ratio Sdr were investigated similarly to a method explained in the example 1. Furthermore, in addition to the evaluation of the abovementioned coating adhesion 1, evaluations of the coating adhesions 3 and 4 shown below were carried out. Results of these are shown in Table 6.

### (Evaluation of the coating adhesion 3)

From each of the obtained steel sheets, a test piece having a width of 40 mm and a length of 100 mm was cut out followed by adhering a cellophane tape (width: 24 mm, manufactured by Nichiban Co., Ltd.) at a position of a length 50 mm, a tape surface was bent inside by 90° followed by unbending, thereafter an amount of Zn adhered when the cellophane tape was peeled was measured as the number of counts by means of X-ray fluorescence analysis. The number of measured counts of Zn was compensated into the number of counts per unit length (1 m) of width of test piece and evaluated according to the following criteria.

### <Evaluation criteria of the coating adhesion 3>

○○: very good (number of counts: 500 or less)
○: good (number of counts: more than 500 and 1000 or less)
Δ: fair (number of counts: more than 1000 and 3000 or less)
×: bad (number of counts: more than 3000)

### (Evaluation of the coating adhesion 4)

From each of the obtained steel sheets, a test piece having a width of 70 mm and a length of 150 mm was cut out, after dipping in rust-preventive oil 550KH (manufactured by Nihon Parkerizing Co. , Ltd.), left in air for 24 hr while standing obliquely, and thus obtained one was used as a test sample. A pressing test was carried out in which in a state where both ends of a test sample 13 were clamped between a die 14 and a wrinkle suppressor 15 that form a bead die 16 such as shown in Fig. 9, from a back surface side of the test sample 13, a punch 17 was pushed in to form a horseshoe shape. A surface of the die was polished with #1000 polishing paper and accretions were cleansed every time. A wrinkle suppressor force P was set at 12 kN and the punching speed was set at 100 mm/min. After the test, the test sample was slightly degreased, followed by adhering a cellophane tape (width: 24 mm, manufactured by Nichiban Corp.). An amount of Zn adhered to the cellophane tape when it was peeled was measured as the number of counts by X-ray fluorescence analysis , and evaluation was carried out according to the following criteria.

### <Evaluation criteria of the coating adhesion 4>

○○: very good (number of counts: 50 or less)
○: good (number of counts: more than 50 and 100 or less)
Δ: fair (number of counts: more than 100 and 300 or less)
×: bad (number of counts: more than 300)

**(Table 6-1)**

| Test sample No. | Steel No. | Concentration of oxygen in a cooling atmosphere until the coating after the recrystallization annealing (vol.%) | Galvannealing condition | | | Galvannealed steel sheet | | | | Evaluation result | | | | Note |
|---|---|---|---|---|---|---|---|---|---|---|---|---|---|---|
| | | | | | | Coating layer | | Base steel sheet | Ratio of fine irregularity in an interface (%) | Coating adhesion 3 | Coating adhesion 1 | | Coating adhesion 2 | |
| | | | Temperature rise speed (°C/s) | Galvannealing temperature (°C) | Holding time (s) | Thickness (µm) | Content of Fe (mass %) | Developed interfacial area ratio Sdr (%) | | | Tensile shear strength | Peeling mode | | |
| 1 | 3A | 0.002 | 20 | 480 | 15 | 6 | 11.0 | 2.6 | 65 | ○○ | ○○ | ○○ | ○○ | |
| 2 | 3A | 0.002 | 25 | 490 | 10 | 3 | 10.5 | 2.3 | 30 | ○○ | ○○ | ○○ | ○○ | |
| 3 | 3A | 0.002 | 25 | 490 | 23 | 6 | 12.9 | 2.7 | 70 | ○ | ○○ | ○○ | ○ | |
| 4 | 3A | 0.001 | 30 | 520 | 25 | 14 | 11.0 | 2.6 | 60 | ○ | ○○ | ○○ | ○○ | |
| 5 | 3B | 0.001 | 25 | 490 | 10 | 7 | 9.2 | 2.2 | 15 | ○○ | ○○ | ○○ | ○○ | |
| 6 | 3C | 0.001 | 30 | 510 | 15 | 11 | 10.5 | 2.4 | 40 | ○ | ○○ | ○○ | ○○ | |
| 7 | 3D | 0.002 | 25 | 490 | 10 | 9 | 10.2 | 2.2 | 20 | ○○ | ○○ | ○○ | ○○ | |
| 8 | 3E | 0.002 | 30 | 520 | 9 | 7 | 10.2 | 2.5 | 50 | ○○ | ○○ | ○○ | ○○ | Example* |
| 9 | 3F | 0.003 | 25 | 490 | 15 | 9 | 11.5 | 2.5 | 40 | ○ | ○○ | ○○ | ○○ | |
| 10 | 3G | 0.002 | 20 | 470 | 25 | 6 | 10.9 | 2.6 | 60 | ○○ | ○○ | ○○ | ○○ | |
| 11 | 3H | 0.002 | 35 | 520 | 15 | 6 | 11.9 | 2.3 | 20 | ○ | ○○ | ○○ | ○○ | |
| 12 | 3I | 0.002 | 20 | 460 | 10 | 4 | 8.9 | 2.1 | 15 | ○○ | ○ | ○○ | ○ | |
| 13 | 3J | 0.002 | 25 | 490 | 15 | 7 | 9.9 | 2.2 | 30 | ○○ | ○○ | ○○ | ○○ | |
| 14 | 3K | 0.002 | 20 | 460 | 30 | 7 | 10.5 | 2.1 | 20 | ○○ | ○○ | ○○ | ○○ | |
| 15 | 3L | 0.002 | 25 | 480 | 20 | 6 | 10.8 | 2.1 | 20 | ○○ | ○○ | ○○ | ○○ | |
| 16 | 3M | 0.002 | 35 | 560 | 4 | 5 | 9.8 | 2.1 | 20 | ○○ | ○○ | ○○ | ○○ | |
| 17 | 3N | 0.002 | 20 | 520 | 20 | 12 | 12.5 | 1.8 | 5 | Δ | Δ | ○ | × | |
| 18 | 30 | 0.002 | 20 | 520 | 25 | 10 | 12.3 | 1.9 | 5 | Δ | ○ | ○ | × | |
| 19 | 3P | 0.002 | 20 | 490 | 15 | 6 | 11.5 | 1.8 | 5 | Δ | Δ | × | ○ | |
| 20 | 3Q | 0.002 | 20 | 520 | 20 | 8 | 12.5 | 1.8 | 5 | × | Δ | Δ | Δ | |
| 21 | 3R | 0.002 | 20 | 490 | 25 | 8 | 11.2 | 1.5 | 0 | Δ | × | × | Δ | |
| 22 | 3S | 0.004 | 30 | 500 | 20 | 10 | 12.5 | 1.5 | 0 | × | × | × | × | |
| 23 | 3T | 0.002 | 20 | 520 | 15 | 7 | 12.2 | 1.4 | 0 | Δ | × | Δ | ○ | Comparative Example |
| 24 | 3U | 0.002 | 30 | 510 | 8 | 7 | 10.2 | 1.6 | 0 | × | × | × | Δ | |
| 25 | 3V | 0.002 | 30 | 480 | 15 | 8 | 9.8 | 1.5 | 0 | ○ | Δ | Δ | ○ | |
| 26 | 3W | 0.002 | 20 | 490 | 20 | 7 | 12.8 | 1.8 | 5 | Δ | ○ | ○○ | Δ | |
| 27 | 3X | 0.001 | 20 | 480 | 12 | 10 | 9.3 | 1.5 | 0 | ○○ | Δ | Δ | ○ | |
| 28 | 3Y | 0.002 | 35 | 490 | 12 | 7 | 10.3 | 1.6 | 0 | × | × | × | Δ | |
| 29 | 3Z | 0.002 | 30 | 470 | 22 | 9 | 11.1 | 1.6 | 0 | × | Δ | Δ | × | |
| 30 | 3D | 0.008 | 25 | 490 | 10 | 9 | 10.2 | 1.9 | 5 | Δ | Δ | Δ | Δ | |

| | | | | | | | | | | | | | | |
|---|---|---|---|---|---|---|---|---|---|---|---|---|---|---|
| * (not according to the invention) | | | | | | | | | | | | | | |

From the evaluation results shown in Table 6, it is found that galvannealed steel sheets of the examples, in comparison with existing steel sheets (comparative examples), are largely heightened in the interfacial strength between the coating layer and the base steel sheet and improved in the coating adhesion.

### Industrial Applicability

Since a galvannealed steel sheet according to the present invention is a galvannealed steel sheet that is remarkably excellent, in comparison with existing ones, in the coating adhesion at an interface between a coating layer and a base steel sheet, in the fields of automobiles, home electric appliances, construction materials and so on, there is no problem of peeling of the coating layer at processing, appearance after the processing is excellent, and sufficient rust resistance can be maintained. Accordingly, an industrially very useful effect in that the high mechanical strength and lighter weight can be attained for all shapes of components can be obtained.

## Claims

1. A galvannealed steel sheet excellent in the coating adhesion, the galvannealed steel sheet comprising a galvannealed layer which is formed on a base steel sheet that
(i) contains, in % by mass, 0.25% or less of C, 0.03 to 2.0% of Si, 0.005 to 0.07% of P, and at least one kind selected from 0.2% or less of Ti, 0.2% or less of Nb and 0.2% or less of V, and
(ii) has a composition satisfying both the equation [C] + [P] ≤ [Si] and the equation [Ti] + [Nb] + [V] ≥ [P], with [C], [Si], [P], [Ti], [Nb] and [V], respectively, meaning the contents (% by mass) of C, Si, P, Ti, Nb and V in the base steel sheet,
wherein, in an interface between the galvannealed layer and the base steel sheet, an irregular portion that has a depth of 10 nm or more at a pitch of 0.5 µm or less is present at least one per 5 µm of a length of the interface, as determined by scanning electron microscopy together with transmission electron microscopy, the depth being defined as the distance in a straight line measured in a height direction between a base that is at a position lowest in height within a reference length and the lower one of a first top and a second top that are at positions highest in height on each of both sides of the base within the reference length, and the pitch being defined as the distance in a straight line measured in a length direction between the first top and the second top within the reference length,
and wherein the base steel sheet contains an oxide of silicon immediate below the interface.

2. The galvannealed steel sheet excellent in the coating adhesion according to claim 1, **characterized in that** the base steel sheet has a composition that further includes, by mass percent, 5 percent or less of Mn, 0.01 percent or less of S and 0.08 percent or less of Al.

3. A method of manufacturing a galvannealed steel sheet as defined in claim 1 or 2, the method comprising the steps of:
(a) heat-treating a base steel sheet that
(i) contains, in % by mass, 0.25% or less of C, 0.03 to 2.0% of Si, 0.005 to 0.07% of P, and at least one kind selected from 0.2% or less of Ti, 0.2% or less of Nb and 0.2% or less of V, and
(ii) has a composition satisfying both the equation [C] + [P] ≤ [Si] and the equation [Ti] + [Nb] + [V] ≥ [P], with [C], [Si], [P], [Ti], [Nb] and [V], respectively, meaning the contents (% by mass) of C, Si, P, Ti, Nb and V in the base steel sheet,
in an atmosphere containing 0.01 to 0.5% by volume of oxygen, having a dew point in the range of -20 to +20°C, the balance being made of nitrogen, and having a temperature in the range of 300 to 500°C so that Si in the steel is not selectively surface oxidized,
(b) heat-treating the base steel sheet obtained from step (a) in a reducing atmosphere containing 3 to 20% by volume of hydrogen, the balance being made of nitrogen, at a temperature in the range of from 750 to 900°C,
(c) cooling the base steel sheet obtained from step (b) to a coating temperature in an atmosphere having an oxygen concentration of 0.005% by volume or less,
(d) dipping the base steel sheet obtained from step (c) in a molten zinc coating bath to form a coating layer, and
(e) heating the base steel sheet obtained from step (d) at a temperature rise speed of 20°C/s or more to a temperature range of 460 to 600°C and holding in the heating temperature range to apply a galvannealing process of the coating layer, wherein the temperature rise speed and the content of Si in the base steel sheet satisfy the equation ST ≥ 3.25/[Si], with ST designating the temperature rise speed (°C/s) and [Si] designating the content (% by mass) of Si in the base steel sheet.

4. The method of manufacturing a galvannealed steel sheet according to claim 3, **characterized in that** the base steel sheet has a composition that further includes, by mass percent, 5 percent or less of Mn, 0.01 percent or less of S and 0.08 percent or less of Al.

## Patentansprüche

1. Verzinktes und wärmenachbehandeltes Stahlblech mit exzellenter Beschichtungshaftung, wobei das verzinkte und wärmenachbehandelte Stahlblech eine wärmenachbehandelte Zinkschicht umfasst, welche auf einem Basisstahlblech ausgebildet ist und das Basisstahlblech
(i) in Masse% angegeben, 0.25% oder weniger an C, 0.03 bis 2.0% an Si, 0.005 bis 0.07% an P, sowie zumindest eines ausgewählt aus 0.2% oder weniger an Ti, 0.2% oder weniger an Nb und 0.2% oder weniger an V enthält und
(ii) eine Zusammensetzung aufweist, welche sowohl die Gleichung [C] + [P] ≤ [Si] als auch die Gleichung [Ti] + [Nb] + [V] ≥ [P] erfüllt, wobei [C], [Si], [P], [Ti], [Nb] bzw. [V] den Gehalt (Masse%) an C, Si, P, Ti, Nb und V in dem Basisstahlblech bezeichnen,
wobei an einer Grenzfläche zwischen der wärmenachbehandelten Zinkschicht und dem Basisstahlblech mindestens alle 5 µm entlang einer Länge der Grenzfläche ein unregelmäßiger Bereich mit einer Tiefe von 10 nm oder mehr und einem Zwischenraum von 0.5 µm oder weniger vorhanden ist, wie mittels Rasterelektronenmikroskopie in Kombination mit Transmissionselektronenmikroskopie bestimmt, wobei die Tiefe als die Entfernung definiert ist, welche in Höhenrichtung auf geradem Weg zwischen einem Basispunkt, der sich am Ort geringster Höhe innerhalb einer Referenzlänge befindet, und der niedrigeren einer ersten Spitze und einer zweiten Spitze, welche sich an den Orten größter Höhe auf jeder der beiden Seiten des Basispunkts innerhalb der Referenzlänge befinden, gemessen wird, und wobei der Zwischenraum als die Entfernung definiert ist, welche in Längsrichtung auf geradem Weg zwischen der ersten Spitze und der zweiten Spitze innerhalb der Referenzlänge gemessen wird,
und wobei das Basisstahlblech ein Oxid von Silizium direkt unterhalb der Grenzfläche enthält.

2. Verzinktes und wärmenachbehandeltes Stahlblech mit exzellenter Beschichtungshaftung nach Anspruch 1, **dadurch gekennzeichnet, dass** das Basisstahlblech eine Zusammensetzung aufweist, welche weiterhin, in Masseprozent angegeben, 5 Prozent oder weniger an Mn, 0.01 Prozent oder weniger an S, und 0.08 Prozent oder weniger an Al umfasst.

3. Verfahren zur Herstellung eines verzinkten und wärmenachbehandelten Stahlblechs, wie es in Anspruch 1 oder 2 definiert ist, wobei das Verfahren die Schritte umfasst:
(a) Wärmebehandeln eines Basisstahlblechs, welches
(i) in Masse% angegeben, 0.25% oder weniger an C, 0.03 bis 2.0% an Si, 0.005 bis 0.07% an P, sowie zumindest eines ausgewählt aus 0.2% oder weniger an Ti, 0.2% oder weniger an Nb und 0.2% oder weniger an V enthält und
(ii) eine Zusammensetzung aufweist, welche sowohl die Gleichung [C] + [P] ≤ [Si] als auch die Gleichung [Ti] + [Nb] + [V] ≥ [P] erfüllt, wobei [C], [Si], [P], [Ti], [Nb] bzw. [V] den Gehalt (Masse%) an C, Si, P, Ti, Nb und V in dem Basisstahlblech bezeichnen,
in einer Atmosphäre, welche 0.01 bis 0.5 Volumen% an Sauerstoff enthält und deren Rest aus Stickstoff besteht, einen Taupunkt im Bereich von -20 bis +20°C besitzt und eine Temperatur im Bereich von 300 bis 500°C aufweist, so dass in dem Stahl befindliches Si nicht selektiv oberflächenoxidiert wird,
(b) Wärmebehandeln des in Schritt (a) erhaltenen Basisstahlblechs in einer reduzierenden Atmosphäre, welche 3 bis 20 Volumen% an Wasserstoff enthält und deren Rest aus Stickstoff besteht, bei einer Temperatur im Bereich von 750 bis 900°C,
(c) Kühlen des in Schritt (b) erhaltenen Basisstahlblechs auf eine Beschichtungstemperatur in einer Atmosphäre, welche eine Sauerstoffkonzentration von 0.005 Volumen% oder weniger aufweist,
(d) Eintauchen des in Schritt (c) erhaltenen Basisstahlblechs in ein Beschichtungsbad aus geschmolzenem Zink, um eine Deckschicht auszubilden, und
(e) Erwärmen des in Schritt (d) erhaltenen Basisstahlblechs mit einer Temperaturerhöhungsgeschwindigkeit von 20°C/s oder mehr auf einen Temperaturbereich von 460 bis 600°C und Halten in dem Erwärmungstemperaturbereich, um die Deckschicht einem Galvannealingprozess zu unterziehen, wobei die Temperaturerhöhungsgeschwindigkeit und der Gehalt an Si in dem Basisstahlblech die Gleichung ST ≥ 3.25/[Si] erfüllen, wobei ST die Temperaturerhöhungsgeschwindigkeit (°C/s) bezeichnet und [Si] den Gehalt (Masse%) an Si in dem Basisstahlblech bezeichnet.

4. Verfahren zur Herstellung eines verzinkten und wärmenachbehandelten Stahlblechs nach Anspruch 3, **dadurch gekennzeichnet, dass** das Basisstahlblech eine Zusammensetzung aufweist, welche weiterhin, in Masseprozent angegeben, 5 Prozent oder weniger an Mn, 0.01 Prozent oder weniger an S, und 0.08 Prozent oder weniger an Al umfasst.

## Revendications

1. Tôle d'acier recuite après galvanisation dont le revêtement présente d'excellentes propriétés d'adhésion, la tôle d'acier recuite après galvanisation comprenant une couche recuite après galvanisation qui est formée sur une tôle d'acier de base qui
(i) contient, en % en masse, 0,25 % ou moins de C, 0,03 à 2,0 % de Si, 0,005 à 0,07 % de P, et au moins une sorte choisie parmi 0,2 % ou moins de Ti, 0,2 % ou moins de Nb et 0,2 % ou moins de V, et
(ii) a une composition satisfaisant à la fois l'équation [C] + [P] ≤ [Si] et l'équation [Ti] + [Nb] + [V] ≥ [P], avec [C], [Si], [P], [Ti], [Nb] et [V], respectivement, désignant les teneurs (% en masse) de C, Si, P, Ti, Nb et V dans la tôle d'acier de base,
dans laquelle, dans une interface entre la couche recuite après galvanisation et la tôle d'acier de base, au moins une portion irrégulière qui a une profondeur de 10 nm ou plus avec un pas de 0,5 µm ou moins est présente par longueur d'interface de 5 µm, telle que déterminée conjointement par microscopie électronique à balayage et par microscopie électronique à transmission, la profondeur étant définie comme la distance dans une ligne droite mesurée dans une direction de la hauteur entre une base qui est à une position la plus basse en hauteur au sein d'une longueur de référence et la plus basse entre un premier sommet et un second sommet qui sont à des positions les plus hautes en hauteur sur chacun des côtés de la base au sein de la longueur de référence, et le pas étant défini comme la distance dans une ligne droite mesurée dans une direction de la longueur entre le premier sommet et le second sommet au sein de la longueur de référence,
et dans laquelle la tôle d'acier de base contient un oxyde de silicium immédiatement en dessous de l'interface.

2. Tôle d'acier recuite après galvanisation dont le revêtement présente d'excellentes propriétés d'adhésion selon la revendication 1, **caractérisée en ce que** la tôle d'acier de base a une composition qui inclut en outre, en pourcent en masse, 5 pourcent ou moins de Mn, 0,01 pourcent ou moins de S et 0,08 pourcent ou moins de Al.

3. Procédé de fabrication d'une tôle d'acier recuite après galvanisation telle que définie dans la revendication 1 ou 2, le procédé comprenant les étapes de :
(a) traitement thermique d'une tôle d'acier de base qui
(i) contient, en % en masse, 0,25 % ou moins de C, 0,03 à 2,0 % de Si, 0,005 à 0,07 % de P, et au moins une sorte choisie parmi 0,2 % ou moins de Ti, 0,2 % ou moins de Nb et 0,2 % ou moins de V, et
(ii) a une composition satisfaisant à la fois l'équation [C] + [P] ≤ [Si] et l'équation [Ti] + [Nb] + [V] ≥ [P], avec [C], [Si], [P], [Ti], [Nb] et [V], respectivement, désignant les teneurs (% en masse) de C, Si, P, Ti, Nb et V dans la tôle d'acier de base,
dans une atmosphère contenant 0,01 à 0,5 % en volume d'oxygène, ayant un point de rosée dans la plage de -20 à +20 °C, le reste étant formé d'azote, et ayant une température dans la plage de 300 à 500 °C de sorte que le Si dans l'acier ne soit pas sélectivement oxydé en surface,
(b) traitement thermique de la tôle d'acier de base obtenue à l'étape (a) dans une atmosphère réductrice contenant 3 à 20 % en volume d'hydrogène, le reste étant constitué d'azote, à une température dans la plage de 750 à 900 °C,
(c) refroidissement de la tôle d'acier de base obtenue à l'étape (b) à une température de revêtement dans une atmosphère ayant une concentration en oxygène de 0,005 % en volume ou moins,
(d) immersion de la tôle d'acier de base obtenue à l'étape (c) dans un bain de revêtement de zinc fondu pour former une couche de revêtement, et
(e) chauffage de la tôle d'acier de base obtenue à l'étape (d) à une vitesse de montée en température de 20 °C/s ou plus jusqu'à une plage de température de 460 à 600 °C et maintien dans la plage de température de chauffage pour réaliser un processus de recuit après galvanisation de la couche de revêtement, dans lequel la vitesse de montée en température et la teneur en Si dans la tôle d'acier de base satisfont l'équation ST ≥ 3,25/[Si], avec ST désignant la vitesse de montée en température (°C/s) et [Si] désignant la teneur (% en masse) de Si dans la tôle d'acier de base.

4. Procédé de fabrication d'une tôle d'acier recuite après galvanisation selon la revendication 3, **caractérisé en ce que** la tôle d'acier de base a une composition qui inclut en outre, en pourcent en masse, 5 pourcent ou moins de Mn, 0,01 pourcent ou moins de S et 0,08 pourcent ou moins de Al.
